

Patented Jan. 8, 1929.

1,698,472

# UNITED STATES PATENT OFFICE.

JOHN R. CAIN, OF WASHINGTON, DISTRICT OF COLUMBIA, ASSIGNOR TO THE RICHARD-  
SON COMPANY, OF LOCKLAND, OHIO, A CORPORATION OF OHIO.

## PROCESS OF MAKING METAL FOILS.

No Drawing.

Application filed May 3, 1926. Serial No. 106,537.

My invention relates to a method of forming metal foils on the surface of an electrolyte.

It has been found that when a metal powder is deposited on an electrolyte, the powder being possessed of the characteristic of floating thereon, that the passing of a current through the resultant film as a cathode will produce a metal foil, capable of self-sustaining.

It is the object of my invention to be herein described to develop a technique of producing foil in this manner, and to describe those methods which apparently produce foils in a regular manner and of best characteristics.

In providing a suitable electrolyte, I have found that neutral or acid electrolytes appear to give best results. Otherwise the general practices of electroplating can be followed, exactly as if the desired metal were to be plated onto an electro-conductive cathode of known character, except that the current densities used in the first stage are higher than usually employed in plating.

The same holds true for the anode, and use of some heat, appears as in electroplating generally to enhance the character of the reaction.

In preparing a floating powder, I prefer either to take a clean dry powder, and treat it with benzol, which is then evaporated off without oxidizing the metal, or I may prepare the powder by precipitating it from an acid salt solution of the metal by the use of a suitable precipitant, such as a metal which will replace the metal of the salt, the acid resulting in a simultaneous production of nascent hydrogen. The precipitated powder when washed and dried will be found to have a floating characteristic of suitable permanence, due, in my opinion to an obscure hydrogen relation to its surface. In the description that follows, I refer to a process using copper powder, and for other metals there will be a like practice varied according to the principles of electroplating.

In any case I prepare an aqueous electrolyte, and deposit the powder thereon from a suitable blower which sprays the dry powder over the surface, where it forms into a seemingly integral film.

The anode is placed below the surface, and coupled to a source of current, and the other terminal is formed by a spongy metallic mass, which is touched to the edges of the floating

film. A suitable blower at one end of the tank, blowing the metal toward the other end will maintain a film like body crowded against the previously deposited metal with which contact is maintained.

I have used with success, a current from one to two amperes per square inch, at a voltage above four volts. When a voltage of twelve volts is used another action is likely to take place which while apparently advantageous, has not been sufficiently investigated by me to be recommended. I have obtained results with over two amperes per square inch, at this stage, and thus do not set a limit as to current.

The turning on of the current results in a very rapid fusion like action of the particles of the metal film, which is the first stage of my process. The use of a spongy cathode at this period is of value because it tends to prevent the formation of hydrogen in excess and thus saves the film from disruption or from being forced away from the cathode.

Also the use of a spongy cathode prevents formation of sponge thereon and on proximate portions of the film. Where sponge forms the film is likely to be broken followed by the sinking thereof.

Also during this period it is advantageous to move the cathode about. In one mechanical arrangement, the cathode can be formed with two branches one of which is moved along one side edge of a vessel containing the powdery film and one along the other edge.

As soon as the film is apparently, to the eye, welded into an integral foil, the second stage of the process will be started, which is nothing but a mere plating action on the welded foil.

At this stage the current densities and practice will be that found most advantageous in regular electroplating for the metal which is to be plated onto the foil.

At this stage the practice will best be, to remove the foil from the first bath, on a suitable screen, and place it in another electrolytic bath, beneath the surface thereof, supported on the screen, and lying between two anodes, the foil being connected as a cathode.

When the foil is thick enough, following the second stage, it is removed from the electrolyte by lifting out the screen, whereupon the foil is washed and dried.

When the operation has progressed sufficiently to make the manipulation of the foil

free of danger of rupture, it will be lifted off of the electrolyte, as by a wire screen, whereupon it is washed and dried.

The temperature of drying should be insufficient to oxidize or tarnish the foil, and after the drying operation the foil is annealed under reducing conditions, at a temperature above that of the reduction temperature of the oxide of the metal. A final 10 treatment by cold rolling between polished metal plates gives a fine finish to the material.

After the foil formation, and before heating and rolling, the foil will usually be dark, 15 and not strong, but with the final treatment it becomes quite strong, and can be used for any purpose to which foil is adapted. In some instances the foil following the second stage will be strong enough to be cold rolled 20 without annealing.

I find that metal powders of one metal can be deposited on an electrolyte of another, such as copper on a zinc electrolyte or copper on a nickel electrolyte. In such cases the primary film is formed of the original metal powder, and during the first stage, the current plates out the other metal between the particles of the film, and assists the integrating thereof into a foil, the whole remaining 25 floating while the first operation continues. The second stage covers this composite foil and apparently the annealing results in the formation of an alloy, which is not usually the case in the foil as formed on the electrolyte. In the first stage some metals, however, 30 will alloy during the primary foil formation.

In all instances the primary foil formed on the electrolyte will float thereon, but will sink if inverted, showing that the underside 40 of the foil retains the floating properties of the original powder.

In the instance of the higher voltages, heretofore referred to, the action is much more

rapid, and appears to show a direct plating of a foil out of the electrolyte onto the surface 45 thereof which discovery I do not include in the present invention.

Having thus described my invention, what I claim as new and desire to secure by Letters Patent, is:—

1. A process of forming metal foil which consists in depositing a metal powder on the surface of an electrolyte, said powder being of a nature to float thereon, and maintaining it in an integral film maintaining contact 55 with the film formed by said powder deposition with a spongy electrode, and providing an anode, and passing an electric current through said electrode and anode.

2. A process of forming metal foil which 60 consists in depositing a metal powder on the surface of an electrolyte, said powder being of a nature to float thereon, and maintaining it in an integral film maintaining contact with the film formed by said powder deposition 65 with an electrode, and providing an anode, and passing an electric current through said electrode and anode, said current being of an amperage of not less than substantially one to two amperes per square 70 inch of metal film surface being acted upon.

3. A process of forming metal foil which consists in depositing a metal powder on the surface of an electrolyte, said powder being of a nature to float thereon, and maintaining 75 it in an integral film maintaining contact with the film formed by said powder deposition with an electrode, and providing an anode, and passing an electric current through said electrode and anode, said current being of an 80 amperage of not less than substantially one to two amperes per square inch of metal film surface being acted upon said current being of a voltage substantially between four and twelve volts.

JOHN R. CAIN.